

- [54] COMBINATION BURNING RATE  
CATALYST AND CURATIVE
- [75] Inventor: David C. Sayles, Huntsville, Ala.
- [73] Assignee: The United States of America as  
represented by the Secretary of the  
Army, Washington, D.C.
- [22] Filed: Feb. 5, 1968
- [21] Appl. No.: 707,358
- [52] U.S. Cl..... 149/19.2, 149/20, 149/21,  
149/44, 102/102
- [51] Int. Cl..... C06d 5/06
- [58] Field of Search ..... 149/19, 20, 42, 44,  
149/11, 2, 21; 102/102

## [56] References Cited

## UNITED STATES PATENTS

3,002,830 10/1961 Barr ..... 149/19

|           |         |                   |           |
|-----------|---------|-------------------|-----------|
| 3,087,844 | 4/1963  | Hudson et al..... | 149/19    |
| 3,109,761 | 11/1963 | Cobb et al.....   | 149/19    |
| 3,305,523 | 2/1967  | Burnside .....    | 149/19 X  |
| 3,322,804 | 5/1967  | Pruett .....      | 149/109 X |

Primary Examiner—Benjamin R. Padgett  
Attorney—Harry M. Saragovitz, Edward J. Kelly,  
Herbert Berl and James T. Deaton

[57] ABSTRACT

Epoxyethylferrocene used as a combination burning rate catalyst and curative in a solid propellant composition.

10 Claims, No Drawings

COMBINATION BURNING RATE CATALYST AND  
CURATIVE  
DEDICATORY CLAUSE

The invention described herein may be manufactured, used, and licensed by or for the Government for governmental purposes without the payment to me of any royalty thereon.

BACKGROUND OF THE INVENTION

This invention relates to a novel burning rate catalyst for use in solid propellant compositions, and in particular to one which also functions as a curative.

Prior art solid propellant compositions have primarily employed cross-linking agents such as tris(methylaziridinyl)phosphine oxide or tris(oxiranyl)para-aminophenol. Other imines and epoxy (oxiranyl) compounds have been used as curatives on occasion. These solid propellant compositions also utilize a burning rate catalyst such as ferrocene or normal-butylferrocene. However, to date there have been no efforts to synthesize a combination burning rate catalyst and curative.

Accordingly, it is the principal object of this invention to provide an improved burning rate catalyst.

It is a particular object of this invention to provide an improved burning rate catalyst which also functions as a crosslinking agent or curative.

SUMMARY OF THE INVENTION

It has been discovered that epoxyethylferrocene can be used as a combination burning rate catalyst and curative in a solid propellant composition.

DESCRIPTION OF THE PREFERRED  
EMBODIMENTS

Epoxyethylferrocene can be used as a combination burning rate catalyst and curative in a solid propellant composition. The solid propellant composition also contains ammonium perchlorate (or other inorganic oxidizer), a metal staple additive such as aluminum, a binder, another burning rate catalyst, if desired, and a processing aid. The binder is formed from a prepolymer reacted with the crosslinking agent in the presence of a polymerization catalyst.

The propellant compositions of this invention are preferably composite (typically having a carboxyl- or hydroxyl-terminated polybutadiene, acrylate, acrylic acid and polybutadiene or polyurethane binder) or composite crosslinkable double-base (typically having a nitrocellulose binder which has been reacted with a plasticizer such as nitroglycerine, and other additives). However, the epoxyethylferrocene can also be used as a substitute for a portion of another oxidizer (e.g., potassium perchlorate or ammonium nitrate) in a double-base or other propellant.

The preferred ingredient concentration ranges of propellant compositions of this invention are (approximate weight percentages):

|                                      |                 |
|--------------------------------------|-----------------|
| Ammonium perchlorate                 | 60-72           |
| Aluminum                             | 2-20 (optional) |
| Binder                               | 9-20            |
| Epoxyethylferrocene                  | 1-15            |
| Three-dimensional crosslinking agent | 0.5-1.5         |

A three-dimensional crosslinking agent and a processing aid (e.g., lecithin) are also present in minute amounts (each about 0.5 percent, or less, by weight).

Of course, the total weight percentages of the ingredients must be 100.

If desired, conventional burning rate catalysts (or other additives) such as copper chromite can be incorporated into the propellant composition in small amounts.

The following table shows a conventional high-burning rate propellant composition (Composition A) compared with Compositions B and C of this invention.

| Ingredient                                   | Composition A | Composition B | Composition C |
|----------------------------------------------|---------------|---------------|---------------|
| Carboxyl-terminated polybutadiene prepolymer | 12.3          | 12.3          | 12.3          |
| 15 Tris(methylaziridinyl)phosphine oxide     | 0.3           | 0.5           | 0.5           |
| Tris(oxiranyl)para-aminophenol               | 0.3           | —             | —             |
| Epoxyethylferrocene                          | —             | 10.0          | 8.5           |
| Normal-butylferrocene                        | 7.0           | —             | —             |
| Iron Linoleate                               | 0.1           | 0.1           | 0.1           |
| Ammonium Perchlorate                         | 66.0          | 63.1          | 64.6          |
| Aluminum                                     | 14.0          | 14.0          | 14.0          |

20 The synthesis of epoxyethylferrocene can be effected by using a one to one molar ratio of acetyl chloride to ferrocene according to the following reaction scheme: acetyl chloride + ferrocene  $\xrightarrow{\text{Friedel-Craft condensation}}$  acetylferrocene  
25 acetylferrocene  $\xrightarrow{\text{Reduction with LiAlH}_4}$  1-ferrocenyl-1-ethanol  
1-ferrocenyl-1-ethanol

30  $\xrightarrow{\text{Dehydration with a mixture of}}$   
acetic and trifluoroacetic anhydrides

Vinylferrocene  $\xrightarrow{\text{Peroxidation with hydrogen peroxide}}$   
35 epoxyethylferrocene

35 By modifying the experimental conditions, bis(epoxyethyl) ferrocene can also be synthesized. This involves using about twice the molar quantities of reactant with ferrocene. Similarly, tris(epoxyethyl)ferrocene may be synthesized by using three times the molar quantities of reactant with ferrocene.

40 45 In general, any lower epoxyalkylferrocene, lower being defined as having one to five carbons in the side-chain of the alkyl group, may be employed in accordance with this invention.

The combination burning rate catalyst and curative of this invention can also be used with solid propellant compositions in which a diisocyanate is used as a chain extender or crosslinking agent. An example of such a diisocyanate is toluene diisocyanate.

50 55 Various other modifications and variations of this invention will become obvious to those skilled in the art in the light of the above teachings, which modifications and variations are within the spirit and scope of this invention.

I claim:

1. A solid propellant composition comprising an inorganic oxidizer selected from ammonium perchlorate, potassium perchlorate, and ammonium nitrate, a binder selected from carboxyl-terminated polybutadiene, hydroxyl-terminated polybutadiene, acrylate, acrylic acid and polybutadiene, polyurethane, and nitrocellulose, and a combination burning rate catalyst and curative comprising a lower epoxyalkylferrocene.

60 65 2. The solid propellant composition of claim 1 wherein said epoxyalkylferrocene is epoxyethylferrocene, bis(epoxyethylferrocene) or tris(epoxyethyl)ferrocene.

3. The solid propellant composition of claim 2 wherein said epoxyalkylferrocene is epoxyethylferrocene.

4. The solid propellant composition of claim 3 wherein said inorganic oxidizer is ammonium perchlorate.

5. The solid propellant composition of claim 4 wherein said binder is formed from a carboxyl-terminated polybutadiene prepolymer.

6. The solid propellant composition of claim 5 10 wherein said prepolymer is crosslinked with tris(methylaziridinyl)phosphine oxide.

7. The solid propellant composition of claim 6 wherein said propellant composition additionally com-

prises a metal staple in an amount of at least about 2 percent by weight.

8. The solid propellant composition of claim 7 wherein said epoxyethylferrocene is present in an amount of from about 1 to 15 percent by weight.

9. The solid propellant composition of claim 8 wherein said metal staple is aluminum.

10. The solid propellant composition of claim 9 wherein said ammonium perchlorate is present in an amount of from about 60 to about 72 percent by weight and wherein said prepolymer is present in an amount of from about 9 to about 20 percent by weight.

\* \* \* \* \*